

166 Patented Aug. 13, 1940

2,211,686

## UNITED STATES PATENT OFFICE

2,211,686

DEPRESSION OF GANGUE DURING  
FLOTATION

Robert B. Booth, Springdale, Conn., assignor to  
American Cyanamid Company, New York,  
N. Y., a corporation of Maine

No Drawing. Application June 28, 1938,  
Serial No. 216,291

13 Claims. (Cl. 209—166)

This invention relates to froth flotation processes and in particular, to the flotation of ores having slimy gangues.

In the past, much difficulty has been encountered with certain ores in which some or all of the gangue constituents have been present as fine slimes which have hindered flotation. The slimes have sometimes been ordinary gangue minerals, such as those of a generally silicious nature, and sometimes have been carbonaceous. While it is often possible to deslime ores prior to treatment by froth flotation, this is not always feasible because in many cases certain components of the slime carry with them recoverable values or, in other cases, it is necessary to grind the feed to a very fine size so that practically all of the feed might be considered as a slime.

The present invention is directed to a froth flotation process in which the gangue is modified, and more particularly the fine gangue, by the addition of a class of reagents so that although it is not removed prior to froth flotation, it does not adversely affect the flotation operation or its adverse effects are to a great extent limited. The present invention is based on the discovery that dyestuffs having solubilizing groupings, and particularly acid dyestuffs containing carboxyl or sulfonic groups or both, exert an action on gangue, preventing interference with froth flotation both in the case of fine silicious gangue and also in the case of carbonaceous gangue, particularly with precious metal ores.

The mechanism of the interference of the gangue with the flotation is probably not the same in all cases, and the present invention is not intended to be limited to any particular theory of action of the finely divided gangue or of the solubilized dyestuffs thereon. In the case of silicious gangue, it is probable that the gangue modifies the surfaces of the values and reduces recovery, whereas the dyestuffs of the present invention appear to so alter or modify the surfaces of the fine gangue particles that they no longer exert this deleterious action or exert it to a very greatly reduced extent. In the case of carbonaceous gangue in carbonaceous precious metal ores, the above factor is not the only one because the carbon also contaminates the concentrate and adversely affects cyanidation of the concentrate which is commonly practiced. In both cases, the present invention greatly reduces the adverse effect of the different types of gangue.

It is an advantage of the present invention that it is applicable to finely divided gangues of

the most varied types of ores, such as precious metal ores, base metal ores, non-metallics and the like. The property of inhibiting the undesirable effects of finely divided gangue appears to be a general one possessed in high degree by all acid dyestuffs, and in considerable degree by dyestuffs which possess solubilizing groups other than sulfonic acid groups. The efficiency of the different dyes will vary to some extent, but they all possess the property of modifying gangue so as to inhibit its undesirable effects. Among the dyes, I have found that water-soluble nigrosine (sulfonated nigrosine) and sun yellow are among the most efficient and at the same time are readily available.

The exact mechanism by which the dyes affect the surfaces of the gangue is not as yet definitely known, and the invention is not intended to be limited to any particular theory of action.

It is an advantage of the present invention that the dyestuffs, while they may be used alone with great effect, can also be combined with other types of gangue modifiers, such as for example lignin sulfonates as described and claimed in the applications of Breerwood, Serial No. 163,302 and Serial No. 163,303 both filed September 10, 1937; dextrin as described and claimed in my copending application, Serial No. 188,075 filed February 1, 1938; crude sugar residues as described and claimed in my copending application, Serial No. 211,811 filed June 4, 1938; and the like. In some of the examples, the use of typical mixtures is described.

The invention will be described in greater detail in conjunction with the following specific examples, the flotation being in every case in standard Fagergren flotation machines except for Example 7 in which a small size special laboratory machine was used.

## Example 1

40

A carbonaceous gold ore from the Mother Lode district containing gold, pyrite, magnetite, arsenopyrite, chalcopyrite, quartz, calcite, muscovite and carbonaceous material, and assaying 0.138 to 0.190 oz. Au per ton, 4.10% Fe, 0.80% C, and about 78% insoluble, was subjected to flotation with and without a dye as gangue modifier. The ore pulp was conditioned with 0.15 lb. per ton of soda ash, 0.21 lb. per ton of copper sulfate pentahydrate, 0.08 lb. per ton of potassium ethyl xanthate, 0.010 lb. per ton of potassium secondary butyl xanthate, 0.10 lb. per ton of a fifty-fifty mixture of sodium diethyl- and dissecondary butyl-dithiophosphates, and 0.062 lb.

lb. per ton of pine oil. The following gangue modifiers were also used: 0.50 lb. per ton of water-soluble nigrosine in test #2, 0.5 lb. per ton of a fifty-fifty mixture of water-soluble nigrosine and a dried molasses residue in test #3, 0.5 lb. per ton of a fifty-fifty mixture of water-soluble nigrosine and calcium lignin sulfonate in test #4, 0.50 lb. per ton of a fifty-fifty mixture of water-soluble nigrosine and yellow corn dextrine in test #5, and no gangue modifier was used in test #1.

netite, limonite and quartz, and assaying 0.308 to 0.327 oz. Au per ton, 0.06% Cu, 2.95% Fe, 0.38% S and about 92% insoluble, was floated. This ore presented a slime interference during flotation. The pulp was conditioned with the following reagents: 0.15 lb. per ton of potassium secondary butyl xanthate, 0.05 lb. per ton of a fifty-fifty mixture of sodium diethyl- and dissecondary butyl-dithiophosphates, and 0.062 lb. per ton of pine oil. The following gangue modifiers were also used: 2.0 lbs. per ton of a stilbene dye,

| 15 | Test No. | Feed  |             | Concentrate     |             |             | Tailing           |                 |             | 15                |    |
|----|----------|-------|-------------|-----------------|-------------|-------------|-------------------|-----------------|-------------|-------------------|----|
|    |          | G.    | Oz. Au, ton | Weight, percent | Ratio conc. | Oz. Au, ton | Percent Au recov. | Weight, percent | Oz. Au, ton | Percent Au recov. |    |
| 20 | 1.       | 602.4 | 0.190       | 14.34           | 7.0/1       | 1.260       | 95.26             | 85.66           | 0.010       | 4.74              | 20 |
|    | 2.       | 603.5 | 0.154       | 5.72            | 17.5/1      | 2.530       | 94.16             | 94.28           | 0.010       | 5.84              |    |
|    | 3.       | 605.0 | 0.138       | 5.62            | 17.8/1      | 2.240       | 91.30             | 94.38           | 0.013       | 8.70              |    |
|    | 4.       | 606.2 | 0.168       | 6.96            | 14.4/1      | 2.280       | 94.64             | 93.04           | 0.010       | 5.36              |    |
|    | 5.       | 604.9 | 0.154       | 6.03            | 14.4/1      | 2.120       | 95.45             | 93.07           | 0.008       | 4.55              |    |

### Example 2

25 A carbonaceous gold ore from South Africa containing pyrite, chalcopyrite, bornite, pyrrhotite, quartz and carbonaceous material, and assaying 0.263 to 0.280 oz. Au per ton, 0.975% S, 1.47% C, and about 91% insoluble, was subjected 30 to flotation with and without a dye as gangue modifier. The ore was conditioned with 0.35 lb.

sun yellow, in test #11; 0.25 lb. per ton of water-soluble nigrosine in test #12; and no gangue modifier was used in test #10. The results of these tests were compared with those obtained by using 2.0 lbs. per ton of soda ash (test #13) and 2.0 lbs per ton of sodium silicate (test #14), two reagents frequently used to overcome slime 30 interference during flotation.

| 35 | Test No. | Feed  |             | Concentrate     |             |             | Tailing           |                 |             | 35                |    |
|----|----------|-------|-------------|-----------------|-------------|-------------|-------------------|-----------------|-------------|-------------------|----|
|    |          | G.    | Oz. Au, ton | Weight, percent | Ratio conc. | Oz. Au, ton | Percent Au recov. | Weight, percent | Oz. Au, ton | Percent Au recov. |    |
| 40 | 10.      | 598.0 | 0.326       | 5.92            | 16.9/1      | 4.620       | 84.05             | 94.08           | 0.055       | 15.95             | 40 |
|    | 11.      | 604.2 | 0.327       | 3.26            | 30.7/1      | 7.960       | 79.20             | 96.74           | 0.070       | 20.80             |    |
|    | 12.      | 605.4 | 0.325       | 1.22            | 82.0/1      | 21.973      | 82.46             | 98.78           | 0.058       | 17.54             |    |
|    | 13.      | 600.0 | 0.308       | 5.17            | 19.3/1      | 4.900       | 82.14             | 94.83           | 0.058       | 17.86             |    |
|    | 14.      | 603.5 | 0.319       | 4.23            | 23.6/1      | 6.200       | 82.13             | 95.77           | 0.060       | 17.87             |    |

45 per ton of potassium secondary butyl xanthate, 0.03 lb. per ton of a fifty-fifty mixture of sodium diethyl- and dissecondary butyl-dithiophosphates, and 0.062 lb. per ton of pine oil. The following gangue modifiers were also used: 1.0 lb per ton of water-soluble nigrosine in test #7, 1.0 lb. per ton of a stilbene dye, sun yellow, in test #8, 1.0 lb. per ton of an anthraquinone dye, alizarin 50 saphirol B, in test #9, and no gangue modifier in test #6.

### Example 4

55 A copper ore containing about 1% Cu and about 64% insoluble, including a large amount of talcose material, was subjected to flotation with and without water-soluble nigrosine as a gangue modifier. In test #16 the ore was conditioned first with 0.25 lb. per ton of water-soluble nigrosine and then with 0.15 lb. per ton of potassium

| 55 | Test No. | Feed  |             | Concentrate     |             |             | Tailing           |                 |             | 55                |    |
|----|----------|-------|-------------|-----------------|-------------|-------------|-------------------|-----------------|-------------|-------------------|----|
|    |          | G.    | Oz. Au, ton | Weight, percent | Ratio conc. | Oz. Au, ton | Percent Au recov. | Weight, percent | Oz. Au, ton | Percent Au recov. |    |
| 60 | 6.       | 605.3 | 0.263       | 19.38           | 5.2/1       | 1.260       | 92.78             | 80.62           | 0.023       | 7.22              | 60 |
|    | 7.       | 601.9 | 0.280       | 4.14            | 24.2/1      | 6.060       | 89.64             | 95.86           | 0.030       | 10.36             |    |
|    | 8.       | 603.5 | 0.265       | 7.71            | 13.0/1      | 3.160       | 92.08             | 92.29           | 0.023       | 7.92              |    |
|    | 9.       | 603.7 | 0.278       | 8.90            | 11.2/1      | 2.870       | 91.73             | 91.10           | 0.025       | 8.27              |    |

### Example 3

65 A gold ore from the Philippine Islands containing gold, pyrite, chalcopyrite, azurite, mag-

secondary butyl xanthate and 0.062 lb. per ton of pine oil; in test #15 no water-soluble nigrosine was used.

| 70 | Test No. | Feed  |            | Concentrate    |             |            | Tailing           |                |            | 70                |    |
|----|----------|-------|------------|----------------|-------------|------------|-------------------|----------------|------------|-------------------|----|
|    |          | G.    | Percent Cu | Percent weight | Ratio conc. | Percent Cu | Percent Cu recov. | Percent weight | Percent Cu | Percent Cu recov. |    |
| 75 | 15.      | 595.9 | 1.10       | 18.78          | 5.3/1       | 5.00       | 85.45             | 81.22          | 0.20       | 14.55             | 75 |
|    | 16.      | 591.7 | 1.12       | 16.34          | 6.1/1       | 5.70       | 83.04             | 83.66          | 0.23       | 16.96             |    |

As demonstrated by the above examples, the use of the dyes as gangue modifiers in the case of both the gold ores and the copper ore resulted in an increased ratio of concentration.

5

*Example 5*

A cement rock from the Lehigh Valley district in Pennsylvania containing calcite, sericite and quartz was ground to about 94% minus 200 mesh. 10 A portion (test #18) was conditioned with 0.5 lb. per ton of water-soluble nigrosine and then floated with 2.0 lbs. per ton of saponified talloel. The results of this test were compared with those obtained in a test with no water-soluble nigrosine (test #17). 15

| Test No. | Feed  |                             | Concentrate     |             |                             | Tailing                          |                 |                             | 20    |
|----------|-------|-----------------------------|-----------------|-------------|-----------------------------|----------------------------------|-----------------|-----------------------------|-------|
|          | G.    | CaCO <sub>3</sub> , percent | Weight, percent | Ratio conc. | CaCO <sub>3</sub> , percent | Percent CaCO <sub>3</sub> recov. | Weight, percent | CaCO <sub>3</sub> , percent |       |
| 17-----  | 598.6 | 71.45                       | 77.38           | 1.3/1       | 75.75                       | 82.04                            | 22.62           | 56.73                       | 17.96 |
| 18-----  | 596.5 | 73.50                       | 83.90           | 1.2/1       | 77.40                       | 88.26                            | 16.09           | 53.70                       | 11.74 |

25 It will be noted that by the use of water-soluble nigrosine, an increase in weight, recovery, grade of concentrate, and recovery of CaCO<sub>3</sub> in concentrate resulted.

*Example 6*

30 Tests have shown that the behaviour of gangue depressants for carbonaceous precious metal ores can be accurately predicted by their action on pure graphite in a small laboratory flotation machine. The results are completely reliable qualitatively and reliable quantitatively with a moderate degree of accuracy. A large number of dyes were tested out in the laboratory machine for their action on graphite slime, the tests being 40 as follows:

|    | Dye name             | Dye class                | Feed, g. | Floated, g. | Tailings, g. | Floated, percent weight | Tailings, percent weight | No. of dye color Index |    |
|----|----------------------|--------------------------|----------|-------------|--------------|-------------------------|--------------------------|------------------------|----|
| 45 | Nigrosine water sol. | Azine                    | 25.1     | 1.3         | 23.8         | 5.18                    | 94.82                    | 865                    | 45 |
|    | do                   |                          | 25.0     | 9.3         | 15.7         | 37.20                   | 62.80                    |                        |    |
|    | Diamond Black PV     | Azo (chrome)             | 25.0     | 1.3         | 23.7         | 5.20                    | 94.80                    | 170                    |    |
|    | Alizarin Saphirol B  | Anthraquinone (acid)     | 25.2     | 0.9         | 24.3         | 3.57                    | 96.43                    | 1054                   |    |
| 50 | Alizarin Sky Blue B  | do                       | 25.2     | 1.8         | 23.4         | 7.14                    | 92.86                    | 1088                   | 50 |
|    | Methyl Cotton Blue   | Triphenylmethane (acid)  | 25.1     | 1.4         | 23.7         | 5.58                    | 94.42                    | 706                    |    |
|    | Patent Blue A        | do                       | 25.2     | 2.4         | 22.8         | 9.52                    | 90.48                    | 714                    |    |
|    | Diamine Green B      | Azo (direct)             | 25.1     | 8.4         | 16.7         | 33.47                   | 66.53                    | 593                    |    |
|    | Spirit Orange        | Azo (acid)               | 25.2     | 2.7         | 22.5         | 10.71                   | 89.29                    |                        |    |
|    | Spirit Red           | do                       | 24.9     | 1.9         | 23.0         | 7.63                    | 92.37                    | 652                    |    |
| 55 | Violamine R          | Xanthene (acid)          | 25.2     | 3.4         | 21.8         | 13.49                   | 86.51                    | 758                    | 55 |
|    | Methyl Violet B      | Triphenylmethane (basic) | 25.1     | 8.2         | 16.9         | 32.67                   | 67.33                    | 680                    |    |
|    | Sun Yellow           | Stilbene (direct)        | 24.7     | 0.7         | 24.0         | 2.83                    | 97.17                    | 620                    |    |
|    | Sap Brown            | Sol. Earth color         | 25.1     | 4.3         | 20.8         | 17.13                   | 82.87                    |                        |    |
|    | Chrysophenine        | Azo (direct)             | 25.2     | 2.5         | 22.7         | 9.02                    | 90.98                    | 365                    |    |
|    | Quinoline Yellow     | Quinoline acid           | 25.1     | 1.2         | 23.9         | 4.78                    | 95.22                    | 801                    |    |
| 60 | Cyanthrol G          | Anthraquinone (acid)     | 25.1     | 1.7         | 23.4         | 6.77                    | 93.23                    | 1077                   | 60 |

The results of these tests indicate that the dyes are effective depressants for graphite.

What I claim is:

1. A method of froth flotation of materials containing floatable metals or metal compounds and finely divided substantially barren non-metalliferous gangue which normally exerts a deleterious action on flotation, said materials being substantially free from molybdenum sulfide, which comprises subjecting the material to flotation in the presence of a collector without removing the gangue and depressing the gangue by means of an effective amount of a dyestuff containing a solubilizing group included in the group consisting of carboxyl, sulfonic, and their salts.

2. A method of froth flotation of materials containing floatable metals or metal compounds and finely divided carbonaceous gangue which normally exerts a deleterious action on flotation, said materials being substantially free from molybdenum sulfide, which comprises subjecting the material to flotation in the presence of a collector without removing the gangue and depressing the gangue by means of an effective amount of a dyestuff containing a solubilizing group included in the group consisting of carboxyl, sulfonic, and their salts. 5

3. A method of froth flotation of materials containing floatable metals or metal compounds and finely divided substantially barren non-metalliferous gangue which normally exerts a deleterious action on flotation, said materials being substantially free from molybdenum sulfide, which comprises subjecting the material to flotation in the presence of a collector without removing the gangue and depressing the gangue by means of an effective amount of water-soluble nigrosine. 10

25 erous gangue which normally exerts a deleterious action on flotation, said materials being substantially free from molybdenum sulfide, which comprises subjecting the material to flotation in the presence of a collector without removing the gangue and depressing the gangue by means of an effective amount of water-soluble nigrosine. 30

4. A method of froth flotation of materials containing floatable metals or metal compounds and finely divided carbonaceous gangue which normally exerts a deleterious action on flotation, said materials being substantially free from molybdenum sulfide, which comprises subjecting the material to flotation in the presence of a collector without removing the gangue and depressing the gangue by means of an effective amount of water-soluble nigrosine. 35

40

gangue by means of an effective amount of water-soluble nigrosine.

5. A method of froth flotation of materials containing floatable metals or metal compounds and finely divided substantially barren non-metalliferous gangue which normally exerts a deleterious action on flotation, said materials being substantially free from molybdenum sulfide, which comprises subjecting the material to flotation in the presence of a collector without removing the gangue and depressing the gangue by means of an effective amount of sun yellow. 65

70

6. A method of froth flotation of materials containing floatable metals or metal compounds and finely divided carbonaceous gangue which nor-

75

- 5 mally exerts a deleterious action on flotation, said materials being substantially free from molybdenum sulfide, which comprises subjecting the material to flotation in the presence of a collector without removing the gangue and depressing the gangue by means of an effective amount of sun yellow.
- 10 7. A method of froth flotation of carbonaceous precious metal ores which comprises carrying out the froth flotation without preliminary removal of carbonaceous gangue and depressing the gangue by means of a dyestuff having solubilizing groups included in the group consisting of carboxyl, sulfonic and their salts.
- 15 8. A method of froth flotation of carbonaceous precious metal ores which comprises carrying out the froth flotation without preliminary removal of carbonaceous gangue and depressing the gangue by means of water-soluble nigrosine.
- 20 9. A method of froth flotation of carbonaceous precious metal ores which comprises carrying out the froth flotation without preliminary removal

of carbonaceous gangue and depressing the gangue by means of sun yellow.

10. A method of froth flotation of non-metals in the presence of finely divided gangue which normally exerts a deleterious action on flotation which comprises carrying out the flotation without removing the fine gangue and depressing the gangue by means of a dyestuff having solubilizing groups included in the group consisting of carboxyl, sulfonic and their salts. 5

11. A method of froth flotation of non-metals in the presence of finely divided gangue which comprises carrying out the flotation without removing the fine gangue and depressing the gangue by means of water-soluble nigrosine. 10

12. A method according to claim 10 in which the material floated is a cement rock raw material. 15

13. A method according to claim 11 in which the material floated is a cement rock raw material. 20

ROBERT B. BOOTH.